

## UNITED STATES PATENT OFFICE

2,111,278

## FERROUS ALLOY

George Charlton, Battle Creek, Mich., assignor to  
Eaton Manufacturing Company, Cleveland,  
Ohio, a corporation of Ohio

No Drawing. Application December 24, 1937,  
Serial No. 181,601

## 1 Claim. (Cl. 75—125)

This invention relates to steel alloys especially adapted for use in lining cylinder sleeves for internal combustion engines and similar uses where it is necessary to have a material that is highly 5 resistant to wear and corrosion, both at normal temperatures and at relatively high temperatures such as 800° F.

The term "wear resisting" as applied to ferrous alloys may have different meanings. For 10 instance, one piece of metal may work in contact with a piece of another metal and the one will show no wear and the other considerable wear. On the other hand, two pieces of different metals can work in contact under the same conditions as 15 in the first instance, and neither will show appreciable wear, although the difference in hardness between the metals may be as great in one instance as in the other. The tendency of a metal to "pick up" particles from another metal with 20 which it is in working contact is aggravated as the temperature is increased.

Alloys which have good wear resistance at room temperature may wear rapidly when the operating temperature increases to the neighborhood of 800° F. The same is true as to corrosion 25 resistance and an alloy which may exhibit satisfactory corrosion resistance at room temperature may corrode rapidly at a temperature in the neighborhood of 800° F.

In order to improve liners for the cylinders of 30 internal combustion engines used in automobiles and aircraft and the like, it has been necessary to produce an alloy which will have improved properties with respect to wear resistance and 35 corrosion in that part of the cylinder which is subjected to the maximum heat. The wear resistance, which is an object of this invention, is 40 the ability of the alloy to resist "pick-up" either under hot or cold conditions, and also show a minimum loss of size when subjected to the working contact of standard piston ring material. The products of combustion of an internal 45 combustion motor are such that when deposited on the walls of a cylinder, which may be dry because of the heat conditions, may, when the motor is idle, have a corrosive effect and it is, therefore, important that the cylinder liner of the motor shall be corrosion resistant. An alloy 50 which will meet the requirements above stated

and produce improved cylinder liners may be made up with a composition as follows:

|              | Per cent      |
|--------------|---------------|
| Carbon       | 1.00 to 3.00  |
| Chromium     | .50 to 10.00  |
| Nickel       | 8.00 to 16.00 |
| Copper       | 3.00 to 6.50  |
| Molybdenum   | .50 to 4.00   |
| Silicon      | .50 to 2.50   |
| Boron        | .25 to 3.00   |
| Manganese    | .25 to 2.00   |
| Sulphur      | not over .5   |
| Phosphorus   | not over .5   |
| Balance iron |               |

It is important that the chromium and molybdenum when taken together shall constitute not less than 4% of the alloy.

The advantages of an alloy made in accordance with this invention, as to wear resistance 20 and corrosion are shown by the following results of comparative tests in which the materials tested were rotated against each other inside a furnace which was heated to a temperature of 800° F. and in an atmosphere of SO<sub>2</sub> gas. The results 25 were as follows:

|              | Loss in<br>thousands  | Corrosion | 30                     |
|--------------|-----------------------|-----------|------------------------|
| Run together | Material #1.....      | .0005     | Very slight corrosion. |
|              | Piston ring iron..... | .00075    | Very slight corrosion. |
| Run together | Material #2.....      | .0003     | Badly corroded.        |
|              | Piston ring iron..... | .0083     | Badly corroded. 35     |

In these tests material #1 was an alloy made in accordance with this invention in which the principal constituents, other than iron, were in 40 the following proportions:

|            | Per cent |
|------------|----------|
| Carbon     | 2.73     |
| Chromium   | 7.70     |
| Nickel     | 13.90    |
| Copper     | 5.88     |
| Molybdenum | 2.02     |
| Silicon    | 1.72     |
| Boron      | 1.23     |

Material #2 is a known commercial alloy of 50

recognized outstanding merit as an abrasion resistor of which the principal constituents, other than iron, are in the following proportions:

|            | Per cent |
|------------|----------|
| 5 Carbon   | 2.32     |
| Manganese  | .61      |
| Silicon    | 1.66     |
| Chromium   | 1.93     |
| Molybdenum | 3.20     |

10 The piston ring iron used in the above tests was a known commercial material that is extensively used in the manufacture of piston rings, the principal constituents of which, other than iron, are in the following proportions:

|               | Per cent |
|---------------|----------|
| Total carbon  | 3.70     |
| Silicon       | 2.70     |
| Manganese     | .60      |
| 20 Phosphorus | .55      |
| Sulphur       | .05      |

25 In addition to the qualities above stated as necessary for an alloy for making cylinder liners it is important that the alloy shall have a relatively low melting point as compared with ordinary steel so that it will be possible to line a steel tube with the alloy by the spinning process in which the molten alloy is deposited on the inside of the tube by the rotation of the latter at high speeds. For this reason the alloy should be in the molten condition at 2300° F. and this temperature is sufficiently below the melting

point of steel to insure that the steel tube will still be strong enough to permit the spinning operation. While in the above method of lining a cylinder it is important that the lining alloy have a melting point not in excess of 2300° F., 5 it is also possible to use the alloy in forming a lining by another method in which the melting point of the alloy is not so vital. In this latter method the molten alloy is poured into a spinning cylinder which is practically at room temperature, and in this case the lining material does not adhere to the cylinder, whereas in the first method the lining material is bonded to the cylinder. 10

An alloy made in accordance with the above 15 formula bears a resemblance to the alloy known as Ni-Resist, in that the nickel and copper proportions are substantially the same in both alloys. However, Ni-Resist is an austenitic cast iron, whereas my improved alloy is not an austenitic cast iron. There is also a difference between the two alloys in that the coefficient of expansion of Ni-Resist is definitely greater than that of my improved alloy. 20

Having thus described my invention, I claim: 25

An alloy steel consisting of 8 to 16% of nickel, 3 to 6.5% copper, 0.5 to 10% chromium, 0.5 to 4% molybdenum, the chromium and molybdenum together being not less than 4%, 0.25 to 2% manganese, 0.25 to 3% boron, 1 to 3% carbon, 30 sulphur not over 0.5%, phosphorus not over 0.5%, silicon 0.5 to 2.5%, and the balance iron.

GEORGE CHARLTON.